

# UNITED STATES PATENT OFFICE.

HANS GOLDSCHMIDT AND OTTO WEIL, OF ESSEN-ON-THE-RUHR, GERMANY, ASSIGNEES  
TO GOLDSCHMIDT THERMIT COMPANY, OF NEW YORK, N. Y., A CORPORATION OF  
NEW JERSEY.

## PROCESS OF MANUFACTURING FERROCHROMIUM.

1,122,907.

Specification of Letters Patent.

Patented Dec. 29, 1914.

No Drawing.

Application filed May 22, 1913. Serial No. 769,179.

*To all whom it may concern:*

- Be it known that we, HANS GOLDSCHMIDT and OTTO WEIL, subjects of the King of Prussia, and residents of Essen-on-the-Ruhr, 5 in the Province of the Rhine, German Empire, have jointly invented certain new and useful Improvements in Processes of Manufacturing Ferrochromium, of which the following is a specification.
- 10 In the specification for our U. S. patent application Serial Number 728,450, filed October 29, 1912 is described a process for increasing the yield of chromium in the aluminothermic production of carbon-free ferro-15 chromium from chrome-iron-ore, such process being based on the observation that in the aluminothermic treatment a much higher percentage of the chromium contained in the chrome-iron-ore is caused to pass into 20 the alloy by the addition of a certain varying percentage of chromium oxid to the mixture of the chrome-iron-ore and aluminum or other reducing metal and then subjecting this mixture to the aluminothermic reaction.
- 25 By this process the yield of chromium from chrome-iron-ore can be increased by about 15 to 20 per cent.

We have found by experiment that various other metal oxides possess the same property which is inherent in chromic oxid, 30 namely, that of allowing or causing a certain percentage of chromium which otherwise would not take a part in the reaction to enter into the same reaction when chrome-35 iron-ore is subjected to the aluminothermic process. The oxids of cobalt, nickel, molybdenum, tungsten, and vanadium all possess this property in a high degree. If, for example, to an aluminothermic mixture consisting of chrome-iron-ore and aluminum a 40 certain proportion of oxid of cobalt is

added and the mixture is ignited the resulting alloy, which of course also contains cobalt, will show a higher percentage of chromium than would be obtained without 45 the addition of oxid of cobalt. The other metal oxids above referred to will act in a similar way.

The peculiarly improved capability of reaction hereinbefore described of the chromium is of very great importance for the production of binary and ternary alloys of chromium with other metals. Owing to the fact that the yield of chromium is considerably increased, these alloys, which are of the 50 greatest importance in steel manufacture, can be produced at a considerably lower price than would be the case if the different metals used, such as chromium and tungsten, had to be prepared first and then alloyed. 55

What we claim is:

1. The process of manufacturing carbon-free ferro-chromium, which consists in mixing materials containing iron and chromium with a metal oxid of the character specified 60 adapted to increase the chromium content of the ultimate product, and subjecting the mixture to the aluminothermic reaction.

2. The process of manufacturing carbon-free ferro-chromium, which consists in mixing chrome-iron-ore with a metal oxid of the character specified adapted to increase the chromium content of the ultimate product, and subjecting the mixture to the aluminothermic reaction. 70

In witness whereof we have hereunto set our hands in the presence of two witnesses.

HANS GOLDSCHMIDT. [L. s.]  
OTTO WEIL. [L. s.]

In the presence of—

HELEN NUFER,  
ALBERT NUFER.